

Dec. 4, 1928.

1,694,179

G. E. JENKS

PROCESS OF REFINING WOOD ROSIN

Filed May 15, 1923

2 Sheets-Sheet 1



*WITNESS.*

Robt R. Kitchel.

George E. Verks  
BY

Frank D. Busson  
ATTORNEY.

Dec. 4, 1928.

1,694,179

G. E. JENKS

PROCESS OF REFINING WOOD ROSIN

Filed May 15, 1923

2 Sheets-Sheet 2



INVENTOR

WITNESS:

Bob W. Kitchel.

George E. Jenks  
by

Frank J. Bauer  
ATTORNEY.

Patented Dec. 4, 1928.

1,694,179

# UNITED STATES PATENT OFFICE.

GEORGE E. JENKS, OF BACCHUS, UTAH, ASSIGNOR TO HEECULES POWDER COMPANY, OF WILMINGTON, DELAWARE, A CORPORATION OF DELAWARE.

## PROCESS OF REFINING WOOD ROSIN.

Application filed May 15, 1923. Serial No. 639,064.

The object of my invention is to so treat wood rosin as to produce a rosin so highly refined that it is adapted for use in sizing the higher grades of paper, in the manufacture of better grades of varnish, and for other purposes for which a high grade rosin is adapted.

A known process of producing wood rosin of a lower grade, and the process that I preferably employ as a preliminary process in the manufacture of more highly refined rosin, consists in grinding wood and stumps from pine trees, placing the wood stock in large digesters, passing steam through the stock and thus driving off a considerable quantity of turpentine, flooding the stock with gasoline or other solvent, thereby extracting certain materials, chiefly rosin, pine oil and various color bodies, passing the gasoline solution, commonly known as "drop liquor", through suitable evaporators, and fractionally removing the gasoline and pine oil. The pine oil produced by the distillation is refined and sold. The recovered gasoline is again used in the process.

The recovered rosin is a marketable product, but is satisfactory for sizing only the lower grades of paper and in making the inferior grades of varnish, and therefore must be marketed at a relatively low price.

A process has been developed by Harry E. Kaiser and Arthur Langmeier, for which they filed an application for patent on the fifteenth day of May, 1923, Serial No. 639,054, whereby the lower grade rosin is subjected to a treatment that greatly improves the color of the rosin and imparts to it generally such high quality, both chemical and physical, as to adapt it for sizing the higher grades of paper and for use in the better grades of varnish. I have so improved the main distillation step of this process as to recover a larger proportion of rosin in the subsequent fractional condensation. In order that my invention may be understood, it will be necessary to describe the above mentioned Kaiser and Langmeier process to which my invention is applicable. It is also necessary to carry out, at least in part, the said process in order to practice the process involving my invention. I shall, therefore, describe the entire process as improved by me and particularly point out that modification of the process involving my invention.

To secure the best results, it is preferred

to preliminarily distill the rosin to remove some of the objectionable coloring matter. The rosin is then heated to a temperature of from 500 to 650° F.—preferably within the higher part of this range. The still vapors are then passed through fractional condensers. If the temperature in the condensers, or one or more of them, is maintained at about 350° F. or over, a practically water-free product results that is comparatively free of rosin oils and pine oils, and there is little danger of the condensed rosin crystallizing. At the end of the system a scrubber is provided to condense the steam and any rosin and rosin oil vapors or mist that pass over the fractional condensers and that, if condensed in the vacuum lines, would clog them up and prevent regular operation.

In the above described process the rosin in the main still is under vacuum and is preferably heated by means of hot oil flowing through tubes with which the rosin is brought into contact or contained in a jacket surrounding a body of rosin. I have discovered that a larger proportion of the rosin can be recovered by injecting into the rosin superheated steam at a temperature approximating the temperature that it is desired to maintain in the still. The superheated steam lowers the temperature of distillation. To secure the degree of heat desired, an independent heating medium, such as the hot oil described, should be used.

In the drawings, which illustrate apparatus for carrying out the major part of the entire process, in its preferable embodiment—

Fig. 1 is a diagrammatic view, in elevation, of that part of the complete rosin refining apparatus comprising the preheater and still.

Fig. 1<sup>A</sup> is a similar view of the remainder of the apparatus, comprising the fractional condensers and scrubbers.

The rosin is first heated in a preheater *a* having a vacuum connection *b* by way of a small condenser *c*. The preheater may be effectively heated by means of a coil *d* through which heated oil is circulated. There are two automatic feeds, one *e* into the preheater and the other *f* from the preheater to the still. The rosin should be heated in the preheater to a temperature of about 480° F. By preheating the rosin, any low boiling coloring matter that may be in the rosin as

it is introduced into the system is taken off and condensed. As different rosins have varying proportions of this low boiling coloring matter, the preliminary distillation will insure substantial uniformity in the material that passes to the main still.

The still *g* is preferably lined with aluminum and the contents thereof are heated by means of hot oil, superheated steam being concurrently injected. The rosin may be heated in batch or continuously. No specific arrangement for transmitting the heat from the oil to the rosin is essential. In the drawings I show a still in which the rosin is so heated in batch by means of a jacket *h*, surrounding the still, through which the heated oil circulates, *i* being the oil inlet and *j* the oil outlet. The superheated steam is introduced by means of a steam pipe *m*. The steam is injected into the body of the rosin. The steam should be at a temperature approximating the temperature that it is desired to maintain in the still.

The rosin should be heated at a temperature well over 500° F. and preferably about 600° or 650° F. The bottom of the still is connected with a vessel *h* to receive the residue.

The rosin vapors are carried off by a pipe *l* through a succession of fractional condensers, which may be of any number, preferably three or four. Three are shown and marked *n*, *o* and *p*. Each condenser is maintained at a predetermined temperature by means of a surrounding jacket *q* in which heated oil is circulated. It is preferred to maintain three condensers *n*, *o* and *p* (where three are used) at temperatures of 400° F., 350° F. and 300° F. respectively.

A high degree of vacuum seems essential to successful rosin distillation. A vacuum of twenty-eight inches of mercury column (if the normal atmospheric pressure is about thirty inches) has been used successfully. It is obvious that with a still higher degree of vacuum the minimum temperature of distillation may be lowered (say 25° F.). When the vacuum drops below twenty-seven inches at the atmospheric pressure specified, the distillation is sluggish. With lower atmospheric pressure, the degree of vacuum would be correspondingly higher. Leakage of air (or oxygen) into the still or condensing system should be avoided, as its effect is to discolor the rosin.

Rosin condensed in the first condenser *n* is of excellent color and of such high quality, both physically and chemically, that it can be used for sizing the highest grade paper, for making the best varnish, and for other purposes. The rosin condensed in the second condenser *o* is of good quality and commands a substantially higher price than the rosin introduced into the system. The rosin condensed in the last condenser *p* is inferior

in quality to that condensed in the other condensers. To produce really high grade rosin, the temperature of the condenser should not be less than 350° F. and should be nearer 400° F. At this temperature is produced a water-free product comparatively free from rosin oil and pine oil, and there is little danger of the condensed rosin crystallizing. By increasing the number of condensers or by heating the condensers to temperatures different from the temperatures herein specified, or by both means, a smaller proportion of the very highest grade rosin, or a larger proportion of rosin of somewhat lower, but still high, grade may be secured. The number of condensers and the temperature regulation will depend upon the grade of rosin that it is desired to obtain and particularly the purpose for which the rosin is intended to be used.

The rosin and rosin oil vapors that escape from the last condenser pass to the solvent scrubber shown. These vapors, which are essentially a mixture of rosin and rosin oil, probably do not amount to over two or three per cent of the rosin distilled. The vapors pass through the return bend pipe condenser *r*, which is water-cooled by means of a distributor *s*. A recirculating stream of solvent (gasoline or kerosene) is maintained inside of the condenser pipes. Without this hydrocarbon solvent, the rosin that would condense in the pipes *r* would not be in sufficient quantity or sufficiently fluid to flow freely. During any single traverse of the condenser pipes, the solvent dissolves much less rosin and rosin vapor than it is capable of absorbing, and it is therefore recirculated until it becomes saturated. The solution of hydrocarbon oil and rosin and rosin oil, mixed with water of condensation, passes to a solvent settling or separating tank *t*, wherein the water settles to the bottom and is withdrawn through the valved pipe *u*. The hydrocarbon oil, with rosin and rosin oil dissolved therein, overflows into a pipe *v* and, by means of a pump *w*, is returned through a pipe *x* to the pipe condenser *r*. As the solvent becomes saturated it is replaced with fresh solvent.

The vacuum in the apparatus may be maintained by connecting the settling tank *t*, through pipe *y*, with vacuum.

Having now fully described my invention, what I claim and desire to protect by Letters Patent is:

1. The process of refining wood rosin which comprises vaporizing the same under a high vacuum by the concurrent action of two heating media, one of which is exteriorly applied and the other of which is superheated steam injected into the body of the rosin, and condensing a portion of the distillate at a temperature not less than about 350° F.

2. The process of refining wood rosin which comprises vaporizing the same under a

high vacuum by the concurrent action of two heating media one of which is exteriorly applied and the other of which is superheated steam injected into the body of the rosin, and 5 fractionally condensing the distillate at temperatures the highest of which does not substantially exceed 400° F.

3. The process of refining wood rosin which 10 comprises preheating the same at a temperature sufficiently above its melting point to drive off low boiling coloring matter and condensing the same, said temperatures being maintained below that required to distill the

rosin, and then heating the rosin to the substantially higher temperature required to distill most of the rosin, said rosin-distilling temperature being established and maintained by the concurrent action of two heating media one exteriorly applied and the other superheated steam injected into the body of 15 20 the rosin; all of said operations being conducted under a high vacuum.

In testimony of which invention, I have hereunto set my hand, at Bacchus, Utah, on this 18th day of April, 1923.

GEORGE E. JENKS.